

Feb. 20, 1962

J. M. BAILEY ET AL  
METHOD AND APPARATUS FOR SIMULTANEOUSLY  
PLATING AND LAPPING  
Filed May 26, 1958

3,022,232



INVENTORS  
JOHN M. BAILEY  
FRED S. ENGELKING  
JAMES L. HOPPER  
JOHN P. JERO

BY *Fryer and Johnson*  
ATTORNEYS

# United States Patent Office

3,022,232

Patented Feb. 20, 1962

1

3,022,232

## METHOD AND APPARATUS FOR SIMULTANEOUSLY PLATING AND LAPPING

John M. Bailey, East Peoria, Fred S. Engelking and James L. Hopper, Peoria, and John P. Jero, Washington, Ill., assignors to Caterpillar Tractor Co., Peoria, Ill., a corporation of California

Filed May 26, 1958, Ser. No. 737,887

5 Claims. (Cl. 204—36)

This invention relates generally to a method and apparatus for automatically finishing a surface to extremely accurate dimensions. More particularly this invention relates to a plating process and the method and apparatus for plating a surface and automatically machining said surface while the object is in the plating solution. Specifically, this invention relates to apparatus for the deposition of material on the surface to be plated and simultaneously, or in combination therewith, for performing a lapping operation on the plated surface while the surface is being plated.

The present invention further relates to a method for developing a precision plated surface by lapping said surface while it is being plated, whereby said surface is produced to true and accurate dimensions by a lap which may be used to produce a plurality of subsequent surfaces of like configuration with virtually no change in the size and finish condition of said subsequently produced surfaces.

It is now the practice to plate articles with certain materials to improve their aesthetic appeal, as well as to protect the surface against wear and corrosion. Depending on the plating material used there are presently known two methods of plate deposition. The most common of these is the electroplating process which utilizes an electric current passing from an anode member to a cathode member (the part being plated) while the part is submerged in a plating solution. Although the process of the present invention may find application in any known method for plating with various materials, the method herein disclosed and described is typical of the electroplating process for the deposition of a wear resistant surface of chromium or a like substance.

In some manufacturing processes worn surfaces of an article have been plated with chromium or other abrasion resistant materials to rebuild the worn areas. These surfaces are subsequently machined to an accurate finish to provide a precision fit between the plated part and a mechanical component operationally arranged in close association with said plated surface. This machining usually comprises the operation of grinding the plated area so that a close working fit is produced between said components.

Although surfaces of many configurations may be produced in various types of articles, the present invention is herein disclosed specifically in connection with the method and apparatus for producing a precision cylindrical bore in a reciprocating plunger pump of the type used in fuel injection systems for internal combustion engines. It is the present practice to machine the bore surface of the pump and finish said bore with a plurality of diamond charged laps that increase in diameter in increments of a few millionths of an inch. Each lap is, therefore, forced into a bore that is slightly smaller than the lap in order to remove the excess material. This operation continues until the largest lap produces a bore surface of desired dimension. The pump bore is then selectively fitted with a pump plunger that has been produced to accurate dimensions by other means.

One obvious disadvantage of this practice is the cost of labor required to select the proper plunger for the bore which will produce a fluid tight fit between the mat-

2

ing parts and the necessity of maintaining these components mated until they are ready for use.

Another disadvantage of the present method of manufacture is the cost of recharging and resizing the diamond charged laps in addition to the tool and labor costs involved in finishing each bore with a plurality of laps of increasing diameter.

Another difficulty presently encountered is in producing a bore surface in a pump barrel wherein said surface is truly cylindrical and capable of restraining the extremely high fluid pressures which are customarily imposed on pumps of the types used in fuel injection systems.

It has heretofore been impossible to perform a machining operation on a plated surface while the part is in the solution with conventional metal laps because the solution contains acids which cause corrosion of the surface of such laps. It is, therefore, an important object of this invention to provide a tool for machining a plated surface which is made of a material that is not affected by acid attack, thereby permitting the machining operation to be conducted while the part is in the plating solution.

The present invention is applicable to and has as another of its objects the provision of a method and apparatus for plating and final machining a surface in the manner described which surface may be continuous or interrupted, external or internal, cylindrical, or of other regular shapes, for the purpose of producing mating parts to predictable dimensions. The process herein disclosed is applicable also to any plating process for producing an extremely precise finish by simultaneously plating and machining a surface.

An important object of this invention is to provide a method and apparatus for manufacturing components of the type described to such a degree of accuracy as to permit interchangeability of parts.

Another object of this invention is to provide a method and apparatus for producing a plated surface to a predictable degree of accuracy during the plating process.

Still another object of this invention is to provide means associated with the plating mechanism to perform a machining operation on the surface being plated during the plating operation.

Still another object of this invention is the provision of a lap member constructed of a non-corrosive material that is harder than the plate deposit which is used to perform a machining operation of the plated surface while the part is being plated.

Still another object of this invention is the provision of a dielectric lap for an electroplating process which comprises means for conducting an electrical current to cause deposition of the plate and perform a lapping operation of the surface plated while the part is in the plating solution.

Another important object of this invention is the provision of a lap member constructed of a ceramic whereby the body of the lap is composed essentially of aluminum oxide and wherein for application in an electroplating process said lap contains anode means for conducting the plating current.

Still another object of the present invention is to provide control means associated with the plating apparatus whereby the temperature of the solution may be regulated or altered to compensate for wear of the surface of the lap so that all such plated surfaces produced by the same lap are virtually dimensionally identical after the parts have cooled.

Further and more specific objects and advantages of this invention will be made apparent in the following specification wherein reference is made to the accompanying drawings.

In the drawings:

FIG. 1 is a diagrammatic view of apparatus representa-

tive of the type required for plating a surface and performing a machining operation thereon while the part is being plated;

FIG. 2 is an enlarged view in elevation of a combination anode and lap member of a preferred structure which is used for producing an extremely accurate plated surface particularly, but not necessarily, by the electroplating process;

FIG. 3 is an enlarged cross-sectional view of the combination anode and lap member taken generally along the lines III—III of FIG. 1;

FIG. 4 is a view in elevation showing a modification of the combination anode and lap member with parts broken away to show the structural details thereof; and

FIG. 5 is an enlarged transverse sectional view of another modification of the anode and lap member.

The apparatus for electroplating disclosed herein should be considered as typical of only one method of liquid bath plating. As seen in FIG. 1 of the drawings, a part 10 to be plated is clamped in a fixture 11 supported on legs 12 or in any suitable manner in the plating solution contained in a tank 13. Part 10 is disposed between plates 14 and 15 of the fixture by suitable nuts threaded to legs 12 to hold the part 10 securely during the plating process. The entire fixture 11 and certain surfaces of part 10 are preferably masked to prevent them from being plated.

Although the surface to be plated may be of various configurations, as heretofore described, the specific surface to be plated herein disclosed is in the form of a cylindrical bore 19 extending through the part 10. Bore surface 19 is machined oversize and finished by reaming or grinding, but it is to be understood that no special precautions need be taken in order to define an accurate finish of the surface 19 prior to it being plated.

In the particular arrangement disclosed in FIG. 1, part 10 is retained in fixture 11 in such a manner that the axis of the bore surface 19 is disposed in a substantially vertical plane.

Finishing of bore surface 19 as it is being plated is performed by a dielectric lap member 21 preferably having a ceramic body of aluminum oxide or other similar material harder than the plating material. The lap is rotated and/or reciprocated by drive means not shown to perform a machining operation on the plate deposition, as will subsequently be described.

Where the plate is deposited by the electroplating process, as shown, part 10 is made of a conducting material so that an electrical current may be conducted thereto from a D.C. current source 16 through a circuit 17 including a contact plate 18 which is held between part 10 and one of the plate members 14 or 15. Anode members in the form of electrical conducting strips 22, such as lead, are used for chrome plating. These anode strips are embedded within flutes 23 formed in the body of lap 21. Flutes 23 may be of various configurations, including straight, or helical flutes as illustrated in FIGS. 1 and 2. Anodes 22 are connected to a collector ring 24 forming a part of a drive coupling illustrated as a double universal joint 28. The electrical circuit is completed by a line 31 leading to brushes 32 which contact a collector ring 25 secured to coupling 28, then through collector ring 24 to cause electrical current to flow through anodes 22.

The lap member 21 illustrated in this specific application of the invention is finished to a very accurate diameter, by any well-known machining process. It will be understood that since the plating solution is usually heated while the part is being plated, the diameter of the lap will not necessarily coincide with the diameter of the finished bore, but the finished bore assumes the proper diameter upon cooling.

In performing the process, lap member 21 is inserted into bore 19 through axially aligned, preferably enlarged openings 33 and 34 provided in plates 14 and 15 respec-

tively. Lap member 21 is rotated and/or reciprocated as previously described by means not shown, and under the influence of the electrical current from source 16, deposits of plate begin to form on the surface 19 of part 10. The build-up of chromium is consistent throughout the surface, substantially duplicating every irregularity existing in surface 19. As the process continues the crests of the irregular surface are contacted by the lap member 21. The relative motion of the lap 21 prevents further build-up of plate in these areas by machining said areas progressively until all the depressions in the surface are relatively completely filled with plate. With this condition obtaining, lap 21 contacts and machines the entire surface to a very smooth and accurate condition.

It is, therefore, possible in the specific example disclosed to define a finished bore to a predictable dimension by the deposition of plate on the surface of an oversized bore and simultaneously, or in combination therewith, produce an accurate dimension by lapping or machining said surface while the part is being plated. It is further possible within the scope of the present invention to produce the external surface of the mating pump plunger by this method to such accurate dimensions as to permit interchangeability of parts. The lap member applied in this instance would of necessity be a female member having the cutting surfaces and anode members in the internal face of a member of substantially tubular shape.

Since the plated surface is lapped while the plate is being deposited, the cutting rate is very light, resulting in a minimum of wear on the lap. Conventional means (not shown) may also be provided to regulate the temperature of the plating solution thereby compensating for the wear of the lap and resulting in the manufacture of subsequent bores that are sized virtually identical to each other with the same lap.

In many instances the rotation and/or reciprocation of the lap will be sufficient to insure adequate circulation of the plating solution between the lap and the part being plated. However, in the arrangement disclosed in FIG. 1 means are provided to furnish a positive flow of the solution between said parts for most efficient plating of the surface. To this end a pump 36 driven in any suitable manner circulates the plating solution from tank 13 through a conduit 37 and pumps the solution through a conduit 38 so as to cause it to flow through the bore defined by the surface 19. The pump discharge conduit 38 is connected to an adapter 39 secured to plate 15 of the fixture as by capscrews 41. Adapter 39 is preferably counterbored as at 42 so as to permit the lap to travel axially therein during its reciprocation and to provide a chamber into which the solution is pumped. The flow of solution is upward between the lap 21 and the surface 19, as illustrated in FIG. 1, and it is discharged through the top end by way of opening 33 in plate 14. The upward flow of solution minimizes the possibility of entrained gases and air pockets becoming trapped along the surface 19 and insures an even deposit of plate thereon.

It will be understood that apparatus may be provided to conduct the solution to the plating area without submerging the part and fixture in the solution as previously described. Where appropriate, as in a machine having a plurality of plating stations, a closed circuit comprising a pump 36, line 38, and a return line (not shown) may be used for circulating the plating solution through each of a plurality of fixtures 11 from a common supply tank.

Although the lap structure described is herein disclosed as a cylindrical member having anode strips embedded within the flutes, it should be noted that various other configurations are likewise suitable for this operation. As illustrated in FIG. 4, a modified structure of the lap is disclosed wherein said lap comprises a plurality of discs 43, made of a similar ceramic material, and alternately disposed discs 44, made of an anode material. These

discs are retained in stacked assembly by a through bolt 46 and secured together by a nut 47 threaded on the end of bolt 46. The ceramic discs 43 are provided with suitable slots 48 defining passages through which the solution is pumped. Simultaneously the peripheral faces of discs 43 lap the plated surface 19 by suitable movement of the lap member 21 as the plate deposit begins to build up sufficiently to contact the lap surface.

Ceramic bodies of the type described are inherently fragile and where applicable a different structure may be used in order to produce a ceramic lap of a more sturdy structure. To this end a modification of the lap structure is disclosed in FIG. 5 wherein a lap body 51 made of a rigid material such as metal is provided with flutes 52 to form the core of the lap. Ceramic material, predominantly aluminum oxide or any substance harder than the plating material, may be bonded to the body of the lap, as at 53, and subsequently machined to an accurate dimension for producing a given size. Furthermore, anode strips 54 made of lead or other suitable materials may likewise be embedded within the flutes of the lap. This structure produces a stronger lap member for performing the process of the present invention. In a construction of this type it may be desirable to mask or insulate the side walls 52a of the flutes 52 to prevent the plating current from shorting out where the core 51 is made of electrical conducting materials.

The lap member of FIG. 5 may have a core of an electrical conducting material which is soft enough, or coated with material which is soft enough, to permit the surface to be charged with particles of a dielectric material (such as aluminum oxide) whereby the plated surface may be lapped while it is in the plating solution. It will be understood that the particle size and the density of the lap surface produced by this process must be controlled to allow the current to pass and still prevent the current from shorting out to the part being plated.

Where the surface to be plated is of a configuration other than cylindrical; as for instance, a square or elliptical bore, a lap of matching configuration carrying anode members is reciprocated relative to the surface while the plate deposition takes place.

Although the specific arrangement as herein disclosed relates to an electroplating process requiring the transfer of an electrical current through anode members in the lap, other lap structures may be used in other plating processes which do not require an electrical current and, therefore, the anode members as well as the electrical circuit will be unnecessary. This type of plating system is commonly referred to as electrodeless plating where the plating material is contained in solution in the plating bath and the plate is deposited by the autocatalytic chemical reduction process. The surface being plated is accurately finished by a ceramic lap while the part is in the plating bath as previously described.

Means (not shown) may also be adapted to the drive controls of this mechanism to determine when the plated surface has been completed. As one example of this type of control, a hydraulic transmission has been used to drive the lap. As the plated surface nears completion the torque required to turn the lap results in higher fluid

pressures which are registered on a torque meter to indicate the load imposed. Experiments have indicated that as the load required to drive the lap rises to a certain level, the process is complete.

The disclosure made herein has been specific to the chromium plating process and for this reason the anode means 22, 44, and 54 have been stipulated as being made of lead. It will be obvious that in plating with other materials, appropriate anode materials, soluble or insoluble, may be substituted for the lead anode material disclosed in this application.

We claim:

1. An article of manufacture for use in performing a machining operation on a surface of a part being electroplated while said part is in contact with an electrolyte comprising a body made of rigid non-conducting grinding material and having flutes formed therein defining land surfaces therebetween, electrical conducting anode means contained in said flutes and recessed from said land surfaces whereby a plating action will take place on a work piece in relative motion to said land surfaces and spaced a slight distance therefrom, and said land surfaces will act to control the depth of plate deposited on said work piece.
2. The article of claim 1 in which the land surfaces are of ceramic material.
3. The article of claim 1 in which the land surfaces and the major portion of the body are formed of ceramic material.
4. The method of producing a surface finish to accurate dimensions which comprises immersing a work piece in an electrolytic bath, moving a lap which has grooves forming intermediate lands conforming to the contour of the surface desired in closely spaced relation to the work piece, and introducing an electric current to said bath through anodes disposed in said grooves to cause plating of the work piece and simultaneously cutting away the deposited plating material until the desired surface conforms in contour to the surface contour of said lands.
5. The method of claim 4 which includes the further step of varying the temperature of the electrolytic bath to compensate for wear of the lap whereby successive work pieces can be produced to the same dimensions with a smaller lap.

45

#### References Cited in the file of this patent

#### UNITED STATES PATENTS

|           |             |               |
|-----------|-------------|---------------|
| 1,271,136 | Cook        | July 2, 1918  |
| 1,721,949 | Edelman     | July 23, 1929 |
| 1,733,404 | Fahrenwald  | Oct. 29, 1929 |
| 1,872,290 | Hitner      | Aug. 16, 1932 |
| 1,886,218 | Olin et al. | Nov. 1, 1932  |
| 1,953,955 | Crouch      | Apr. 10, 1934 |
| 2,871,177 | Comstock    | Jan. 27, 1959 |
| 2,920,026 | Kistler     | Jan. 5, 1960  |

#### FOREIGN PATENTS

|         |               |               |
|---------|---------------|---------------|
| 712,314 | Great Britain | July 21, 1954 |
| 18,643  | Great Britain | Aug. 18, 1900 |
| of 1899 |               |               |

60